

Jan. 14, 1936.

T. MISHIMA

2,027,994

MAGNET STEEL CONTAINING NICKEL AND ALUMINUM

Filed Jan. 20, 1932

2 Sheets-Sheet 1



INVENTOR.

T. Mishima  
BY: Marks & Clark

ATTORNEYS.

Jan. 14, 1936.

T. MISHIMA

2,027,994

MAGNET STEEL CONTAINING NICKEL AND ALUMINUM

Filed Jan. 20, 1932

2 Sheets-Sheet 2

Fig. 7



T. Mishima  
INVENTOR

By: Marks & Clark  
Attest.

## UNITED STATES PATENT OFFICE

2,027,994

MAGNET STEEL CONTAINING NICKEL  
AND ALUMINIUMTokushichi Mishima, Ochiai-machi,  
Toyotama-gori, Tokyo, JapanApplication January 20, 1932, Serial No. 587,822  
In Japan March 9, 1931

4 Claims. (Cl. 175—21)

The invention relates to a strong permanent magnet comprising 5 to 40% nickel, 7 to 20% aluminium and the remainder iron. It has for its object to economically obtain a permanent magnet which possesses an extremely high coercive force and a strong residual magnetism without being quenched after casting and preserves these qualities without being influenced by thermal changes and mechanical shocks and has 10 small specific gravity and non-corrosive property.

Heretofore many magnet steels, such as tungsten-, chrome-, and chrome manganese-steels have been known. However, in order to obtain 15 the best magnetic property, they must necessarily be quenched, and consequently they often suffer from deformation and quenching cracks. Besides, not only their coercive force and residual magnetism are low, but also during the use of 20 these magnets their coercive force and residual magnetism decrease gradually.

The high-cobalt steel alone has a considerably high coercive force and strong residual magnetism. However, it has the disadvantages that 25 it must be forged and heat-treated which is difficult, and in addition its cost is very high so that its general uses are greatly hindered.

Nickel is a ferromagnetic substance while aluminium is a paramagnetic one, and it has been 30 known to all that these metals give no beneficial effects upon the coercive force and residual magnetism of steels when they are added to the latter individually.

Now nickel steels containing 5-30% nickel are 35 called "irreversible steel" by which is meant that they become transformed at appreciably higher temperatures on heating than on cooling. That is, the  $Ac_2$  point (the temperature at which magnetism is lost on heating) is considerably higher 40 than the  $Ar_2$  point (the temperature at which magnetism begins to obtain on cooling), and the difference amounts to over 400° C. For this reason, when cooling high-nickel steels from high 45 temperature above the  $Ac_2$  point, the  $Ar_2$  transformation points are suppressed and the steels become non-magnetic at room temperature due to the retention of  $\gamma$ -iron. This is the reason why scientists insist upon, and metallurgists give assent, to the fact that the nickel steels can not be 50 used for magnet steels.

According to the invention it is possible to economically obtain magnet steels which possess an extremely high coercive force and a strong residual magnetism without being quenched, and

preserve these qualities permanently without being influenced by thermal changes and mechanical shocks. For this purpose the invention provides for a permanent magnet containing iron as its chief component, with the addition of 5-40% 5 nickel and 7-20% aluminium.

In the accompanying drawings, Figs. 1 to 6 explain the principle upon which the invention is based; Figs. 1 to 3 being curves showing the relation between the temperature and the intensity 10 of magnetization; Figs. 4 to 6 show the relation between the thermal dilatation and the temperature corresponding to Figs. 1 to 3; and Fig. 7 shows the demagnetizing curves, that is the fourth quadrant of the hysteresis curves comparing the magnetic properties of the steel according 15 to the invention and those of other known steels.

Now, the reason why according to the invention a permanent magnet having high coercive force and strong residual magnetism can be obtained 20 without being quenched, is explained with reference to the accompanying drawings.

Take a nickel alloy or an "irreversible nickel alloy" having such relation between the intensity of magnetization and temperature as shown in 25 Fig. 1, and add to it a certain amount of aluminium. Then, as shown in Fig. 2 the point  $Ar_2$  at which magnetism begins to obtain on cooling comes near the point  $Ac_2$  at which magnetism commences to be lost on heating; by then increasing the amount of aluminium and attaining a proper amount, the point  $Ar_2$ , as shown in Fig. 3, coincides with the point  $Ac_2$  the "irreversible steel" thus changing into a "reversible one". It will also be seen from Fig. 4, that the "irreversible 35 nickel steel" has the point  $Ac_3$ , where the steel changes from  $\alpha$  state to  $\gamma$  state on heating, considerably higher than the point  $Ar_3$ , where the steel changes from  $\gamma$  state to  $\alpha$  state on cooling. And the temperature-difference between  $Ac_3$  and 40  $Ar_3$  is in fact over 400° C.

According to the invention the phenomena are entirely different and proceeds as follows: with the gradually increased amount of aluminium, the point  $Ar_3$  comes, as shown in Fig. 5, nearer and nearer to the point  $Ac_3$ , and with such a definite addition as corresponds to Fig. 3, the point  $A_3$  disappears entirely as shown in Fig. 6. Thus the "irreversible nickel steel" can be changed into a "reversible one" by the addition of aluminium, while the transformation point  $A_3$  entirely disappears. It can therefore easily be seen that according to the invention high coercive force and strong residual magnetism are obtained without 50 55

the steel being quenched after casting, or by annealing it at proper temperature after casting.

Several examples showing the compositions and magnetic properties of the alloy according to the invention are illustrated below:

| 10 | Alloy No. | Chemical composition (per cent) |        |          | Magnetic properties         |                                 |
|----|-----------|---------------------------------|--------|----------|-----------------------------|---------------------------------|
|    |           | Iron                            | Nickel | Aluminum | Coercive force (Hc) (gauss) | Residual magnetism (Br) (gauss) |
| 15 | I         | Rest.                           | 18.0   | 10.0     | 120                         | 9,100                           |
|    | II        | 65.3                            | 24.5   | 10.0     | 240                         | 9,600                           |
|    | III       | 57.0                            | 30.8   | 12.0     | 430                         | 9,400                           |

In Fig. 7, the curves 1, 2 and 3 show the characteristic properties of the magnet steels corresponding to the above alloys I, II and III, while the curves 4, 5 and 6 show those of tungsten-, chrome-, and chrome manganese-steels respectively. As clearly seen in this figure, all the magnet steels previously known have poor coercive force, whereas the steel according to the invention has an extremely high coercive force Hc and a strong residual magnetism Br. Therefore the product of these two qualities (Br  $\times$  Hc) is obviously far greater than those of other known steels. It is noted that the presence of carbon of below 1.5% and/or a small amount of impurities does not materially affect the magnetic properties of the alloy according to the invention.

As described above, according to the invention the nickel steel, formerly entirely disregarded as a permanent magnet steel, can now be easily changed into a strong permanent magnet steel by an addition of a proper amount of aluminium, which is a cheap material. The steel

will be furnished with an extremely high coercive force and a strong residual magnetism without being quenched. By this means, therefore, the defect that the known magnetic steel must necessarily be subjected to deformation and quenching-cracks when quenched, is completely eliminated. The alloy according to the invention will be applied for general uses, and in particular for permanent magnets of precise measuring apparatus and generators, and other various kinds of measuring devices.

Permanent magnets made of alloys which embody additional elements such as vanadium, molybdenum, tungsten, manganese, copper, cobalt and chromium and which have similar properties necessary for permanent magnets form the subject-matter respectively of the following divisional applications: 673,796, May 31, 1933; 35,207, Aug. 7, 1935; 35,208, Aug. 7, 1935; 673,795, May 31, 1933; 35,209, Aug. 7, 1935; 9,685, March 20 6, 1935.

In this case also it is noted that the presence of carbon of below 1.5% and/or a small amount of impurities does not materially affect the magnetic properties of the alloy.

I claim:

1. A permanent magnet comprising 5 to 40% nickel, 7 to 20% aluminium and the remainder iron.

2. A permanent magnet comprising 5 to 40% nickel, 7 to 20% aluminium and the remainder substantially iron.

3. A permanent magnet comprising 5 to 40% nickel, 7 to 20% aluminium, from trace to 1.5% carbon and the remainder iron.

4. A permanent magnet comprising 5 to 40% nickel, 7 to 20% aluminium, from trace to 1.5% carbon and the remainder substantially iron.

TOKUSHICHI MISHIMA.